

# UNITED STATES PATENT OFFICE.

FRANK G. BREYER, ALBERT E. HALL, AND GEORGE R. WALTZ, OF PALMERTON, PENNSYLVANIA, ASSIGNORS TO THE NEW JERSEY ZINC COMPANY, OF NEW YORK, N. Y., A CORPORATION OF NEW JERSEY.

## PRODUCTION OF METAL OXIDS AND OTHER COMPOUNDS OF METALS.

1,322,090.

Specification of Letters Patent. Patented Nov. 18, 1919.

No Drawing.

Application filed July 12, 1918. Serial No. 310,440.

*To all whom it may concern:*

Be it known that we, FRANK G. BREYER, ALBERT E. HALL, and GEORGE R. WALTZ, all citizens of the United States, residing at 5 Palmerton, Pennsylvania, have invented certain new and useful Improvements in the Production of Metal Oxids and other Compounds of Metals; and we do hereby declare the following to be a full, clear, and 10 exact description of the invention, such as will enable others skilled in the art to which it appertains to make and use the same.

This invention relates to the production of metal oxids or other compounds of metals 15 volatilized by the Wetherill process.

Metallic oxids, such, for example, as zinc 20 oxid and leaded zinc oxid, as well as other compounds of metals volatilized by the Wetherill process, such, for example, as basic lead sulfate or sublimed lead, have heretofore been more or less extensively produced by the so-called Wetherill process. In speaking of metals volatilized by the 25 Wetherill process, we intend to describe and cover such metals as are volatilizable at the temperatures attainable in the Wetherill process, and for the sake of brevity, we shall hereinafter designate these metals as volatilizable metals. In the case of certain of 30 such metals, the final or desired compound or compounds thereof are the result of a sequence of actions in which the metalliferous materials of the charge are reduced, the reduced metal volatilized and then oxidized or otherwise compounded, while in 35 other cases a metal compound may be directly volatilized, with or without subsequent oxidation or compounding.

By the expression "Wetherill process" as 40 we have used the same herein is to be understood the furnacing step of the process for producing metal oxids or other compounds of volatilizable metals in which a charge of the metalliferous material mixed 45 with a reducing agent and spread on an ignited bed of fuel is subjected to a combustion supporting blast of draft and brought to a sufficiently high temperature to reduce the metalliferous materials and 50 volatilize the reduced metal or metals (and (or) to volatilize a metal or a metal compound or compounds) without bringing the charge to a condition where it becomes impervious to the blast or draft, the entire 55 charge being supported on a furnace hearth

or grate designed to hold it without letting any considerable part drop through, and the worked-off material being discharged as a clinker or sinter. The "furnacing step" is independent of the subsequent treatment of 60 the laden furnace gases and of the collection of the metal compound or compounds.

As a typical example of the Wetherill process, as heretofore usually practised, we will briefly describe the customary procedure in the commercial production of zinc 65 oxid, including leaded zinc oxid. The furnacing step is generally carried out in a furnace having a broad expanse of horizontal grate or hearth roofed over with an arch, 70 and associated with appropriate instrumentalities for permitting the passage therethrough and into the charge, by either a blast or draft, of a combustion supporting gas. It is customary to first charge upon 75 the furnace grate or hearth a layer of "buckwheat" anthracite coal (which is thereupon ignited, usually by the residual heat of the furnace) and by means of a forced blast or draft of air to bring this initial layer of 80 coal to well-developed combustion. Upon this layer of "bed coal" is then charged the customary mixture or "working charge" 85 characteristic of the Wetherill process, that is to say, a mixture of finely divided reducing coal with the finely divided zinciferous (or zinciferous and plumbiferous) material, such as zinc silicate, roasted zinc blends, roasted so-called "mixed sulfids" of zinc and lead, spelter retort residues, or 90 other reducible zinc-containing or zinc-and-lead containing material at the disposal of the operator. The forced air draft is continued, and, when the familiar flames of 95 greenish tint, known as "zinc candles," begin to make their appearance above the upper surface of the charge, indicating that the reduction and volatilization of the zinc and its oxidation to the form of fume is well under way, the products of combustion 100 carrying the zinc oxid fume and other volatilized metallic compounds are conveyed through the customary cooling flues, etc., to the bag-room wherein, in a cooled condition, they filter through the bags and pass 105 off into the atmosphere, leaving the fume collected in the interior of the bags, from which it is removed at convenient intervals. The furnace operation is continued until the production of fume therefrom in appre- 110

ciable quantity ceases, whereupon the residual charge, which is, to a large extent, sintered together, is broken up by long-handled rabbles and pried up and lifted or scraped 5 out through the furnace doors into a receiving pit, or the like, preparatory to the starting of a new operation. The coal or other carbonaceous material of the charge serves the two-fold purpose of furnishing 10 a reducing agent for effecting the reduction of the metalliferous materials of the charge and of furnishing, by combustion, the necessary degree of heat to bring these materials to the reducing temperature characteristic 15 of the process.

As thus ordinarily practised, the above-described furnace operation is attended with certain defects interfering with its full efficiency. Prominent among these defects is 20 the inevitable tendency to the formation of blow-holes or craters at various regions of the charge. Working or rabbling of the charge to break up these blow-holes involves considerable labor, and, in addition, the 25 formation of blow-holes causes waste of fuel and inefficiency in the recovery of values. A further defect of the above-described furnace operation is that the forced draft tends to project into the free space above the 30 charge more or less dust, and thus dusting is further aggravated by the rabbling operations. This dust contaminates the fume and damages its color and marketability. These and many of the other defects of the 35 above-described furnace operation as heretofore generally practised are overcome to a very remarkable extent by modifying the heretofore customary practice in accordance with the improvements described in the application for Letters Patent of the United 40 States of Frank G. Breyer, James A. Singmaster and Albert E. Hall, Serial No. 270,179, filed January 8, 1919. These improvements consist in supplying either or 45 both the bed fuel and the working charge to the furnace hearth in the form of briquets. The improved results attendant upon this modification in the prior customary practice are described in detail in the aforementioned application.

We have discovered that a further decided improvement in the efficiency of the aforementioned furnace operation can be secured by appropriately modifying the relative 50 proportions of fuel, including reducing agent, in the working charge and bed fuel in accordance with the principles hereinafter explained. Thus, briefly, we have discovered that when the greater proportion of 55 the total fuel of the charge is placed in the form of briquets in the bed fuel, rather than in the working charge as has heretofore been customary, a very complete working-off of the volatilizable metal values is 60 effected. The relatively deep bed of fuel 65

briquets when in full combustion imparts to the superposed working charge a highly reducing atmosphere and a sufficiently high and very uniform temperature whereby 70 90% or more of the volatilizable metals may be recovered from the metalliferous material of the charge, as compared with recoveries of about 70% under the heretofore customary furnace practice with unbriqueted charges and recoveries of from 75 80 to 85% with briqueted charges as described in the aforementioned Breyer-Singmaster-Hall application.

The residual charge from the hereinbefore described furnace operation (with unbriqueted charges) consists of a more or less sintered mass containing the ash of the consumed fuel, unconsumed fuel and the worked-off metalliferous material. These various materials are more or less mixed together and their mixed condition seriously prejudices subsequent treatment of the residue and the separation and recovery therefrom of such valuable materials as it usually contains. When this heretofore customary practice is modified by supplying the usual working charge mixture to the furnace hearth in the form of briquets, the worked-off charge is still a mixture of ash, unconsumed fuel and worked-off metalliferous 90 material. By placing the greater proportion of the total fuel of the charge in the bed fuel in the form of briquets, and by supplying the working charge, with its correspondingly reduced content of fuel and reducing agent, in the form of briquets, we very materially reduce the amount of combustible material associated with the metalliferous material of the working charge and thereby enable the working charge briquets 100 to retain for the most part their original form and shape, whereby the worked-off ore or metalliferous briquets may be readily separated from the clinkered residue of the bed fuel briquets. At the same time, the 110 amount of ash associated with the worked-off ore briquets is of such small amount that these worked-off briquets can be subsequently treated for the recovery of further metallic values without serious difficulty. 115

In the customary commercial practice of the Wetherill process, the total carbonaceous material in the entire charge, including the bed fuel and the working charge mixture, is several times greater than the theoretical amount required to reduce the compounds of the volatilizable metals in the charge. It has heretofore been the general practice to place the greater proportion of the total carbonaceous material 120 of the entire charge in the working charge mixture. For example, when operating with the well known Franklin furnace zinc oxide ores, it is customary to place from about 125 fifteen (15) to twenty-five (25) per cent. of 130

the total carbonaceous material of the entire charge in the bed fuel, while the remaining eighty-five (85) to seventy-five (75) per cent. of the total carbonaceous material is 5 mixed with the ore to form the working charge. In general terms, the layer of bed fuel is approximately one inch in depth of thickness, while the working charge mixture is spread over the ignited bed fuel in a layer 10 from about five (5) to seven (7) inches in depth or thickness.

We have discovered that a very considerable proportion of the carbonaceous or other combustible material can be withdrawn from 15 the working charge and placed in the bed fuel when the bed fuel is supplied to the furnace hearth in the form of briquets. Thus, for example, when operating with Franklin furnace zinc oxid ores, we have obtained 20 excellent results by placing from about seventy-five (75) to eighty-five (85) per cent. of the total carbonaceous material of the entire charge in the bed fuel and supplying this bed fuel to the furnace hearth 25 in the form of briquets. The remaining twenty-five (25) to fifteen (15) per cent. of the total carbonaceous material is then admixed with the ore to form the working charge. The working charge is also pref- 30 erably briqueted and spread on the ignited bed fuel briquets.

In carrying out the invention, the briquetted bed fuel is charged onto the furnace hearth in any appropriate manner, ignited 35 and brought to full combustion by passing a combustion-supporting gas, such as air, into the bed fuel briquets. The working charge is then spread onto the ignited bed of fuel briquets, and the resulting effluent 40 is withdrawn from the furnace and appropriately treated for the removal and collection of the metallic compounds contained therein. In working with Franklin furnace zinc oxid ores, we have secured very satis- 45 factory results by charging the briquetted bed fuel in a layer of approximately five (5) to six (6) inches in depth or thickness, and spreading onto the ignited layer of these bed fuel briquets a layer of working 50 charge briquets of approximately four (4) to five (5) inches in depth or thickness.

When the compounds of the volatilizable metals of the working charge have been worked-off to the desired extent, the residual 55 charge may be withdrawn or discharged from the furnace in any suitable manner. This residual charge consists of a relatively thin layer of clinker on which rests the worked-off ore briquets. During the process 60 the bed fuel briquets undergo substantially complete combustion, and are discharged as a clinkered ash. On the other hand, the physical form of the briquetted working charge is not materially altered and for the 65 most part the worked-off ore briquets retain

their original shape with only incipient fusion.

The bed fuel briquets may be prepared by compressing finely divided coal, together with a suitable binder, such, for example, as 70 the concentrated waste sulfite liquor of the sulfite paper pulp industry. Various forms and grades of carbonaceous material are available for the bed fuel briquets. Thus, for example, anthracite coal below the No. 75 3 buckwheat size, such as No. 4 buckwheat, colliery washings, "dirt" coal, "dust" coal, as well as coke breeze, may be utilized in the production of the bed fuel briquets. The bed fuel briquets are of such size and shape 80 as to materially reduce the resistance to the combustion supporting gas, and nevertheless to supply such a substantially uniform substratum for the support of the superposed working charge as to give free access therethrough and practically equal distribution thereto of the combustion supporting gas. To this end, the bed fuel briquets, as well as the working charge briquets, should be of substantially uniform size, and preferably 85 of such shape that they roll or tumble easily over one another. Thus, we have found the so-called pillow block, eglette, rounded pillow block, over-stuffed pillow, and similar shapes well suited to the purposes of the 90 invention.

While the working charge consisting of a mixture of the metalliferous material and an appropriate reducing agent may be supplied to the ignited layer of bed fuel briquets in 100 an unbriqueted form, we prefer to briquet the working charge because of the many attendant advantages. Furthermore, we wish it to be understood that the metalliferous material may be briqueted alone, 105 without briquetting the reducing agent, or the reducing agent may be briqueted alone without briquetting the metalliferous material, or the reducing agent and the metalliferous material may be separately briqueted. 110 However, our preferred practice is to briquet a mixture of the metalliferous material and the reducing agent.

The reducing agent of the working charge may be of any suitable kind, and while we 115 now prefer to employ carbonaceous material as the reducing agent, it will be understood by those skilled in the art that reducing agents other than carbonaceous materials are available for the purpose of the invention. 120 One of the advantages of employing a briquetted reducing agent in any of the forms hereinbefore described is that it permits the use of carbonaceous materials of cheaper grades and finer mesh, such as anthracite 125 coal of finer mesh than No. 3 buckwheat, colliery washings, dust coal, coke breeze and the like.

The bed fuel briquets and the working charge briquets may be prepared in any 130

appropriate manner. We have found the procedure described in the aforementioned application of Frank G. Breyer, James A. Singmaster and Albert E. Hall, Serial No. 5 270,179, for preparing similar fuel and working charge briquets well adapted for the purposes of our present invention. This procedure involves generally the steps of mixing the material to be briqueted with a 10 suitable binder, such as concentrated waste sulfite liquor of 30° Baumé, molding the mixture into briquets of the desired size and shape, and drying or baking the briquets at a temperature of approximately 15 200° C., so as to impart to them the desirable amount of resistance to crumbling and breaking so that they may be freely subjected to the rough handling incident to storing them, conveying them to the furnace, and incident to charging them into 20 the furnace either by hand or otherwise. In the case of the briqueted metalliferous material, it is also desirable that the briquets possess such resistance to crumbling and breaking as to substantially maintain 25 their form during the entire furnacing operation, so that they are for the greater part discharged from the furnace in substantially their original physical form.

30 When practising the Wetherill process in accordance with the principles of our present invention, the residual charge consists of a more or less clinkered coal ash, resulting from the combustion of the bed fuel briquets, 35 and a residue, resulting from the working-off of the metalliferous charge. When, as in the preferred embodiment of the invention, the metalliferous material of the working charge is supplied to the furnace hearth in 40 the form of briquets, this residue contains the worked-off ore briquets in substantially their original physical form. Some of the working charge briquets will almost inevitably become broken or crushed in the preliminary handling and furnacing operation, 45 but these briquets for the greater part retain their original physical form. After the furnacing operation, these briquets are remarkably hard and almost coke-like in their 50 physical characteristics, and are readily separated from the clinkered coal ash of the bed fuel briquets.

55 This capability of readily separating the worked-off metalliferous or ore briquets from the ash of the fuel briquets is of especial advantage when the worked-off ore briquets are to be subjected to further treatment for the recovery of valuable metals not volatilizable by the Wetherill process. As a result 60 of practising the Wetherill process in accordance with our present invention, this advantage is greatly augmented by the fact that the worked-off metalliferous briquets contain at most only a relatively small 65 amount of ash. Where the working charge

briquets consist of a mixture of metalliferous material and carbonaceous reducing agent, the worked-off briquets will contain, in addition to the worked-off metalliferous material, the ash from the consumed carbonaceous reducing agent as well as the unconsumed portion of the reducing agent. The ash is composed principally of silica and alumina, and is generally objectionable in any subsequent treatment of the worked-off 70 metalliferous briquets. Thus, for example, in those instances in which the worked-off metalliferous briquets are smelted in a blast furnace for the production of spiegeleisen a certain amount of fluxing agents is necessary 75 for slagging off the ash present in the worked-off metalliferous briquets, and when this amount of ash is relatively large an objectionably large amount of fluxing agent is required, with the resultant production of 80 an objectionably large amount of slag. By the practice of our present invention the main bulk, for example, around eighty-five (85) per cent. of the ash of the total carbonaceous material of the charge is in the 85 clinker resulting from the combustion of the bed fuel briquets, and the worked-off metalliferous briquets are consequently contaminated with only a relatively small amount of 90 ash. On account of this relatively slight 95 ash contamination of the worked-off metalliferous briquets, as well as on account of their physical properties, these briquets are peculiarly well adapted for subsequent treatment in blast furnaces. In addition to retaining their original form, these briquets are moreover of a porous character, due to the removal of the volatilizable metals therefrom, and this porous property of the 100 worked-off briquets is also of advantage in 105 their subsequent treatment.

As a typical instance of the practice of the invention, we will briefly describe a particular charge and the manner of working the same. The charge was made up of the 110 well known Franklin furnace zinc oxid ores and dust coal. Approximately eighty-five (85) per cent. of the total coal of the charge was briqueted with concentrated waste sulfite liquor as the binder, in the manner previously described. The remaining fifteen (15) per cent. of the total coal was mixed with the ore (in the proportion of about ninety (90) parts of ore to ten (10) parts of coal dust) to which was added about three (3) per cent. of concentrated waste sulfite liquor as a binder and the mixture was then briqueted and the briquets baked, as previously described. The fuel briquets were first charged onto the perforated hearth of 115 the present day customary type of zinc oxid furnace and ignited by the residual heat of the preceding furnacing operation. A thin layer of fuel briquets was first charged, and after these had been well ignited, the re- 120 125 130

mainder of the fuel briquets were charged, producing a layer of bed fuel of about six (6) inches in depth. When this layer of bed fuel had reached full combustion, the briquetted working charge was spread thereon, producing a superposed layer of working charge briquets of about five (5) inches in depth. During these operations, a blast of air was maintained through the perforated grate, 10 and when active reduction of the zinciferous material of the charge began, the effluent from the furnace was conducted to the oxid drums and thence to the bag-room in the usual manner. The temperature of the 15 charge was maintained at from about 1100° C. to about 1250° C., and the fume emitting period was of substantially four hours' duration.

The residual charge consisted of a more or 20 less clinkered coal ash of about three-fourths ( $\frac{3}{4}$ ) to one and one-half (1 $\frac{1}{2}$ ) inches in thickness, resulting from the combustion of the fuel briquets, and worked-off metalliferous or ore briquets retaining for the greater 25 part their original form with only incipient fusion. This residual charge was withdrawn from the furnace by hand and the worked-off ore briquets separated from the remainder of the residual charge for subsequent treatment.

The zinc oxid produced was of a very high 30 grade, free from grit or specks and very bright. The recovery of zinc was remarkably high, being about ninety (90) per cent. 35 on the original zinc content of the raw ore.

While we have hereinbefore specifically 40 described the invention by reference to the production of zinc oxid, including leaded zinc oxid, we wish it to be understood that the invention is applicable to the production of other metal compounds of the volatilizable metals. In particular, we contemplate the 45 production of basic lead sulfate or sublimed lead by the method of the invention. In general, the procedure for the production of sublimed lead is substantially the same as hereinbefore described, substituting, of course, an appropriate plumbiferous material for the zinciferous material. Thus, for 50 example, the bed fuel is briquetted in the manner hereinbefore described, and contains the bulk or greater proportion of the total carbonaceous or other combustible material of the entire charge. The working charge 55 consists of a mixture of finely divided galena or native lead sulfid and carbonaceous material preferably briquetted as hereinbefore described. The working charge is spread on the ignited layer of bed fuel briquets and 60 upon reaching the reaction temperature, the lead sulfid is reduced and (or) volatilized and subsequently oxidized to lead sulfate and lead oxid thus forming the so-called basic lead sulfate.

65 The effluent containing the sublimed lead

is withdrawn from the furnace and the metallic product collected in any appropriate manner. The worked-off plumbiferous briquets containing as they do a relatively small amount of contaminating ash may be advantageously subjected to any appropriate subsequent treatment for the recovery of the non-volatilizable metals of the original metalliferous material. As the source of plumbiferous material, we may use a high 70 grade of native lead sulfid suitably crushed and jigged to free it from accompanying gangue material, or we may use lead sulfid concentrates, such as flotation concentrates, or other appropriate plumbiferous-containing material, with proper additions of sulfur in the form of pyrite, galena, brimstone or other suitable sulfur-carrying agents, whenever there is a lack of sulfur in the charge to properly sulfate the fume. 75

The relatively deep layer of bed fuel, when in complete combustion, provides a substantially incandescent sub-stratum of carbonaceous material of appreciable depth upon which rests the metalliferous material of the 80 working charge. By appropriately controlling the amount of combustion supporting gas introduced into the bed fuel, complete utilization of the oxygen of such gas can be effected during its passage through the bed 85 fuel and the superposed metalliferous material can be subjected to a strong and effective reducing atmosphere. This reducing atmosphere may be so controlled as to materially reduce the amount of reducing agent 90 in the working charge, and in certain instances may even eliminate the necessity of admixing any reducing agent with the metalliferous material of the working charge. 95

We claim:

1. In the production by the Wetherill process of metal oxids or other compounds of volatilizable metals, the step of supplying to the furnace hearth a relatively deep layer 100 of bed fuel in the form of briquets, together with the steps of spreading on the ignited layer of bed fuel briquets a working charge containing metalliferous material and a reducing agent; substantially as described. 115

2. In the production by the Wetherill process of metal oxids or other compounds of volatilizable metals, the step of supplying to the furnace hearth a relatively deep layer 120 of bed fuel in the form of briquets, together with the step of spreading on the ignited layer of bed fuel briquets a working charge containing metalliferous material and a briquetted reducing agent; substantially as described. 125

3. In the production by the Wetherill process of metal oxids or other compounds of volatilizable metals, the step of supplying to the furnace hearth a relatively deep layer 130 of bed fuel in the form of briquets, together

with the step of spreading on the ignited layer of bed fuel briquets a working charge containing briquetted metalliferous material and a reducing agent; substantially as described.

4. In the production by the Wetherill process of metal oxides or other compounds of volatilizable metals, the step of supplying to the furnace hearth a relatively deep layer 10 of bed fuel in the form of briquets, together with the step of spreading on the ignited layer of bed fuel briquets a working charge composed of a briquetted mixture of metal-liferous material and a reducing agent; sub- 15 stantially as described.

13 substantially as described.

5. In the production by the Wetherill process of metal oxides or other compounds of volatilizable metals, the step of supplying to the furnace hearth a layer of bed fuel containing the greater part of the total combustible material of the entire charge in the form of briquets, together with the step of spreading on the ignited layer of bed fuel briquets a working charge containing metalliferous material and a reducing agent, substantially as described.

20

25

6. In the production by the Wetherill process of metal oxides or other compounds of volatilizable metals, the step of supplying 30 to the furnace hearth a layer of bed fuel containing the greater part of the total combustible material of the entire charge in the form of briquets, together with the step of spreading on the ignited layer of bed fuel 35 briquets a working charge containing metaliferous material and a briquetted reducing agent; substantially as described.

7. In the production by the Wetherill process of metal oxides or other compounds of volatilizable metals, the step of supplying to the furnace hearth a layer of bed fuel containing the greater part of the total combustible material of the entire charge in the form of briquets, together with the step of spreading on the ignited layer of bed fuel briquets a working charge containing briquetted metalliferous material and a reducing agent; substantially as described.

8. In the production by the Wetherill  
50 of metal oxides or other compounds of vola-  
tilizable metals, the step of supplying to  
the furnace hearth a layer of bed fuel con-  
taing the greater part of the total com-  
bustible material of the entire charge in the  
55 form of briquets, together with the step of  
spreading on the ignited layer of bed fuel  
briquets a working charge composed of a  
briqueted mixture of metalliferous material  
and a reducing agent; substantially as de-  
60 scribed.

9. In the production by the Wetherill process of metal oxides or other compounds of volatilizable metals, the step of supplying to the furnace hearth a layer of bed fuel

containing from about 75% to about 85% of the total combustible material of the entire charge in the form of briquets, together with the step of spreading on the ignited layer of bed fuel briquets a working charge containing metalliferous material and a reducing agent; substantially as described. 65 70

10. In the production by the Wetherill process of metal oxides or other compounds of volatilizable metals, the step of supplying to the furnace hearth a layer of bed fuel containing from about 75% to about 85% of the total combustible material of the entire charge in the form of briquets, together with the step of spreading on the ignited layer of bed fuel briquets a working charge containing metalliferous material and a briquetted reducing agent; substantially as described.

11. In the production by the Wetherill process of metal oxides or other compounds of volatilizable metals, the step of supplying to the furnace hearth a layer of bed fuel containing from about 75% to about 85% of the total combustible material of the entire charge in the form of briquets, together with the step of spreading on the ignited layer of bed fuel briquets a working charge containing briquetted metalliferous material and a reducing agent; substantially as described. 85 90 95

scribed.

12. In the production by the Wetherill process of metal oxides or other compounds of volatilizable metals, the step of supplying to the furnace hearth a layer of bed fuel containing from about 75% to about 85% of the total combustible material of the entire charge in the form of briquets, together with the step of spreading on the ignited layer of bed fuel briquets a working charge composed of a briquetted mixture of metalliferous material and a reducing agent; substantially as described.

13. In the production of sublimed lead by the Wetherill process, the step of supplying to the furnace hearth a relatively deep layer of bed fuel in the form of briquets, together with the step of spreading on the ignited layer of bed fuel briquets a working charge containing plumbiferous material and a reducing agent; substantially as described. 110 116

14. In the production of sublimed lead by the Wetherill process, the step of supplying to the furnace hearth a relatively deep layer of bed fuel in the form of briquets, together with the step of spreading on the ignited layer of bed fuel briquets a working charge containing plumbiferous material and a briquetted reducing agent; substantially as described. 120 125

15. In the production of sublimed lead by the Wetherill process, the step of supplying to the furnace hearth a relatively deep

- layer of bed fuel in the form of briquets, together with the step of spreading on the ignited layer of bed fuel briquets a working charge containing briqueted plumbiferous material and a reducing agent; substantially as described.
16. In the production of sublimed lead by the Wetherill process, the step of supplying to the furnace hearth a relatively deep 10 layer of bed fuel in the form of briquets, together with the step of spreading on the ignited layer of bed fuel briquets a working charge composed of a briqueted mixture of plumbiferous material and a reducing agent; substantially as described.
17. In the production of sublimed lead by the Wetherill process, the step of supplying to the furnace hearth a layer of bed fuel containing the greater part of the total combustible material of the entire charge in the 20 form of briquets, together with the step of spreading on the ignited layer of bed fuel briquets a working charge containing plumbiferous material and a reducing agent; substantially as described.
18. In the production of sublimed lead by the Wetherill process, the step of supplying to the furnace hearth a layer of bed fuel containing the greater part of the total combustible material of the entire charge in the 30 form of briquets, together with the step of spreading on the ignited layer of bed fuel briquets a working charge containing plumbiferous material and a briqueted reducing agent; substantially as described.
19. In the production of sublimed lead by the Wetherill process, the step of supplying to the furnace hearth a layer of bed fuel containing the greater part of the total combustible material of the entire charge in the 40 form of briquets, together with the step of spreading on the ignited layer of bed fuel briquets a working charge containing briqueted plumbiferous material and a reducing agent; substantially as described.
20. In the production of sublimed lead by the Wetherill process, the step of supplying to the furnace hearth a layer of bed fuel containing the greater part of the total combustible material of the entire charge in the 50 form of briquets, together with the step of spreading on the ignited layer of bed fuel briquets a working charge composed of a briqueted mixture of plumbiferous material and a reducing agent; substantially as described.
21. In the production of sublimed lead by the Wetherill process, the step of supplying to the furnace hearth a layer of bed fuel 60 containing from about 75% to about 85% of the total combustible material of the entire charge in the form of briquets, together with the step of spreading on the ignited layer of bed fuel briquets a working charge
- containing plumbiferous material and a reducing agent; substantially as described.
22. In the production of sublimed lead by the Wetherill process, the step of supplying to the furnace hearth a layer of bed fuel containing from about 75% to about 85% of the total combustible material of the entire charge in the form of briquets, together with the step of spreading on the ignited layer of bed fuel briquets a working charge containing plumbiferous material 70 and a briqueted reducing agent; substantially as described.
23. In the production of sublimed lead by the Wetherill process, the step of supplying to the furnace hearth a layer of bed fuel 80 containing from about 75% to about 85% of the total combustible material of the entire charge in the form of briquets, together with the step of spreading on the ignited layer of bed fuel briquets a working charge 85 containing plumbiferous material and a briqueted reducing agent; substantially as described.
24. In the production of sublimed lead by the Wetherill process, the step of supplying to the furnace hearth a layer of bed fuel containing from about 75% to about 85% of the total combustible material of the entire charge in the form of briquets, together with the step of spreading on the ignited 95 layer of bed fuel briquets a working charge composed of a briqueted mixture of plumbiferous material and a reducing agent; substantially as described.
25. In the production of metal oxids or other compounds of volatilizable metals, the step of supplying to the furnace hearth a relatively deep layer of bed fuel in the form of briquets, together with the step of spreading on the ignited layer of bed fuel 100 briquets a working charge containing metalliferous material; substantially as described.
26. In the production of metal oxids or other compounds of volatilizable metals, the step of supplying to the furnace hearth a 110 relatively deep layer of bed fuel, together with the step of spreading on the ignited layer of bed fuel a working charge containing briqueted metalliferous material; substantially as described.
27. In the production of metal oxids or other compounds of volatilizable metals, the step of supplying to the furnace hearth a relatively deep layer of bed fuel in the form of briquets, together with the step of 115 spreading on the ignited layer of bed fuel briquets a working charge containing briqueted metalliferous material; substantially as described.
28. In the production of metal oxids or other compounds of volatilizable metals, the step of supplying to the furnace hearth a relatively deep layer of bed fuel, together 120

with the step of spreading on the ignited layer of bed fuel a working charge composed of a briqueted mixture of metalliferous material and a reducing agent; substantially as described.

29. In the production of metal oxids or other compounds of volatilizable metals, the step of supplying to the furnace hearth a layer of bed fuel containing in excess of 10 25% of the total combustible material of the entire charge in the form of briquets, together with the step of spreading on the ignited layer of bed fuel briquets a working charge containing metalliferous material; substantially as described.

30. In the production of metal oxids or other compounds of volatilizable metals, the step of supplying to the furnace hearth a layer of bed fuel containing in excess of 20 25% of the total combustible material of the entire charge in the form of briquets, together with the step of spreading on the ignited layer of bed fuel briquets a working charge containing briqueted metalliferous material; substantially as described.

31. In the production of metal oxids or other compounds of volatilizable metals, the step of supplying to the furnace hearth a layer of bed fuel containing from about 30 75% to about 85% of the total combustible material of the entire charge in the form of briquets, together with the step of spreading on the ignited layer of bed fuel briquets a working charge containing metalliferous material; substantially as described.

32. In the production of metal oxids or other compounds of volatilizable metals, the step of supplying to the furnace hearth a layer of bed fuel containing from about 40 75% to about 85% of the total combustible material of the entire charge in the form of briquets, together with the step of spreading on the ignited layer of bed fuel briquets a working charge containing briqueted metalliferous material; substantially as described.

33. In the production of sublimed lead by the Wetherill process, the step of supply to the furnace hearth a relatively deep layer 50 of bed fuel in the form of briquets, together with the step of spreading on the ignited layer of bed fuel briquets a working charge containing plumbiferous material; substantially as described.

34. In the production of sublimed lead by the Wetherill process, the step of supplying to the furnace hearth a relatively deep layer 60 of bed fuel, together with the step of spreading on the ignited layer of bed fuel a working charge containing briqueted plumbiferous material; substantially as described.

35. In the production of sublimed lead by the Wetherill process, the step of supplying to the furnace hearth a relatively deep layer 85 of bed fuel in the form of briquets, together

with the step of spreading on the ignited layer of bed fuel briquets a working charge containing briqueted plumbiferous material; substantially as described.

36. In the production of sublimed lead by 70 the Wetherill process, the step of supplying to the furnace hearth a relatively deep layer of bed fuel, together with the step of spreading on the ignited layer of bed fuel a working charge composed of a briqueted mixture of plumbiferous material and a reducing agent; substantially as described.

37. In the production of sublimed lead by 80 the Wetherill process, the step of supplying to the furnace hearth a layer of bed fuel containing in excess of 25% of the total combustible material of the entire charge in the form of briquets, together with the step of spreading on the ignited layer of bed fuel briquets a working charge containing 85 plumbiferous material; substantially as described.

38. In the production of sublimed lead by 90 the Wetherill process, the step of supplying to the furnace hearth a layer of bed fuel containing in excess of 25% of the total combustible material of the entire charge in the form of briquets, together with the step of spreading on the ignited layer of bed fuel briquets a working charge containing briqueted plumbiferous material; substantially as described.

39. In the production of sublimed lead by 100 the Wetherill process, the step of supplying to the furnace hearth a layer of bed fuel containing from about 75% to about 85% of the total combustible material of the entire charge in the form of briquets, together with the step of spreading on the ignited layer of bed fuel briquets a working charge containing 105 plumbiferous material; substantially as described.

40. In the production of sublimed lead by 110 the Wetherill process, the step of supplying to the furnace hearth a layer of bed fuel containing from about 75% to about 85% of the total combustible material of the entire charge in the form of briquets, together with the step of spreading on the ignited layer of bed fuel briquets a working charge 115 containing briqueted plumbiferous material; substantially as described.

41. In a process for volatilizing and oxidizing metal values involving the blowing of air into a bed containing combustible material and a mixture of the metal-bearing material and a reducing agent under conditions which will leave the worked-off charge as a clinker and which will produce a volatile fume, the step of supplying the combustible 120 material in the form of a relatively deep layer of briquets; substantially as described.

42. In a process for volatilizing and oxidizing metal values involving the blowing of air into a bed containing combustible ma- 125

terial and a mixture of the metal-bearing material and a combustible reducing agent under conditions which will leave the worked-off charge as a clinker and which 5 will produce a volatile fume, the step of supplying the combustible material in the form of a relatively deep layer of briquets containing the greater part of the total combustible material of the entire charge; sub- 10 stantially as described.

43. In a process for volatilizing and oxidizing metal values involving the blowing of air into a bed containing the metal-bearing material and combustible material under 15 conditions which will leave the worked-off charge as a clinker and which will produce a volatile fume, the step of supplying at least part of the combustible material in the form of a relatively deep layer of briquets; sub- 20 stantially as described.

44. In a process for producing sublimed lead involving the blowing of air into a bed containing combustible material and a mixture of the metal-bearing material and a

combustible reducing agent under conditions 25 which will leave the worked-off charge as a clinker and which will produce a volatile fume, the step of supplying the combustible material in the form of a relatively deep 30 layer of briquets containing the greater part of the total combustible material of the entire charge; substantially as described.

45. In a process for producing sublimed lead involving the blowing of air into a bed containing the metal-bearing material and 35 combustible material under conditions which will leave the worked-off charge as a clinker and which will produce a volatile fume, the step of supplying at least part of the combustible material in the form of a relatively 40 deep layer of briquets; substantially as described.

In testimony whereof we affix our signatures.

FRANK G. BREYER.  
ALBERT E. HALL.  
GEORGE R. WALTZ.

Corrections in Letters Patent No. 1,322,090.

It is hereby certified that in Letters Patent No. 1,322,090, granted November 18, 1919, upon the application of Frank G. Breyer, Albert E. Hall, and George Waltz, of Palmerton, Pennsylvania, for an improvement in "Production of Metal Oxids and other Compounds of Metals," errors appear in the printed specification requiring correction as follows: Page 2, line 30, for the word "thus" read *this*; page 6, line 49, claim 8, after the word "Wetherill" insert the word *process*; page 7, lines 100, 108, 116, 125, claims 25, 26, 27, 28, and page 8, lines 6, 16, 26, 36, claims 29, 30, 31, 32, after the word "production" insert the words *by the Wetherill process*; same page, line 48, claim 33, for the word "supply" read *supplying*; and that the said Letters Patent should be read with these corrections therein that the same may conform to the record of the case in the Patent Office.

Signed and sealed this 30th day of December, A. D., 1919.

[SEAL.]

M. H. COULSTON,  
*Acting Commissioner of Patents.*

Cl. 75—19.